

June 2, 1936.

D. T. SMITH

2,042,639

PROCESS OF COOKING PITCH

Filed Feb. 28, 1933

Fig. 1.



Fig. 2.



INVENTOR

Daniel T. Smith

BY

John Sibley

ATTORNEY

Patented June 2, 1936

2,042,639

# UNITED STATES PATENT OFFICE

2,042,639

## PROCESS OF COOKING PITCH

Daniel Tollie Smith, Wylam, Ala., assignor to  
The Barrett Company, New York, N. Y., a cor-  
poration of New Jersey

Application February 28, 1933, Serial No. 658,912

3 Claims. (Cl. 202—6)

This invention relates to the coking of hydro-carbon material, and more particularly, to the coking of coal tar pitch in a beehive oven to produce hard, firm, metallurgical coke.

5 In the Hall patent, No. 1,650,126, of November 22, 1927, there is disclosed and claimed a procedure of coking coal tar pitch in a beehive oven which results in the production of a hard, firm, metallurgical coke. The process of this patent 10 yields an improved coke of extremely high carbon content and extremely low in volatiles, ash, and sulphur. The invention of this application is in the nature of a specific improvement on the procedure of the Hall patent.

15 As a result of extensive development work, I have found that the quality of coke produced by coking coal tar pitch or other hydrocarbons is materially affected by the temperature of the oven being charged. In order to produce a high 20 grade of metallurgical coke, so-called "finger coke", it is necessary to cool the oven before charging. Should the temperature of the oven be reduced more than is necessary in cooling the oven after the completion of the coking of one 25 charge, it will frequently be found that the coke obtained from the next charge of coke will have green ends and an excessively high volatile content. On the other hand, if the oven is not cooled sufficiently, the coking of the next charge of pitch 30 will result in semi-foamy or foamy coke and not hard, firm, dense coke. One possible explanation for the latter phenomenon is that if the floor of the oven is not properly cooled, it will retain substantial amounts of heat, and upon introduction 35 of a fresh charge of pitch into the oven, this heat rushes into the coal tar pitch, causing foaming thereof and premature coking of portions of the charge and the formation of spongy, foamy coke.

40 I have found that the quenching and removal of coke from the oven when the temperature within the oven reaches a definite predetermined range results in the oven having a suitable temperature for the reception and coking of a subsequent pitch charge and that by quenching and removing successive charges within this definite 45 temperature range, hard, firm, dense coke of good quality is uniformly produced.

45 In accordance with my invention, the coking 50 of a charge of six tons of coal tar pitch of 400° F. melting point in a beehive oven, of the type shown on the drawing having a floor diameter of 12'—6" and an altitude of 8'—0½", is discontinued when the temperature at the floor of the 55 oven reaches a temperature of from 1500° F. to

2000° F., determined by means of an electrical pyrometer, the thermo-couple of which is placed directly on the floor of the oven near the center of the floor. When the temperature at the floor of the beehive oven reaches the point hereinabove indicated, the coke is quenched with an amount 5 of water just sufficient to quench the coke, resulting in a lowering of the temperature at the floor of the oven to a temperature of from 600° F. to 800° F. Thereafter, the coke is withdrawn and 10 a fresh charge of pitch is introduced into the oven, the high temperatures prevailing therein initiating combustion of the volatiles in the pitch. The introduction of the pitch results in a further 15 lowering of the temperature in a beehive oven. During the introduction of the pitch and for some time thereafter, the temperature may drop about 200° F. Thereafter, when the combustion within the oven becomes more pronounced, the temperature rises gradually so that at the end of about 20 forty (40) hours, the temperature reaches from about 1500° F. to about 2000° F. and the coking is completed. At this point, the coking is discontinued, 25 the coke quenched and withdrawn, and a fresh charge of pitch introduced, etc.

25 In practice, it has been found, however, that the placing of a thermo-couple on the floor of the oven in direct contact with the coke will not ordinarily give a reliable record of the temperature at the floor of the oven during the coking of succeeding charges since the temperature in proximity to the thermo-couple within the oven is affected by how the coke cracks and the exact position of the thermo-couple with respect to the cracks. In order to obtain a reliable indication 30 of the temperature within the oven and at the floor thereof, it is preferred to place the thermo-couple beneath the floor out of contact with the coke. In the case of a circular beehive oven having a floor layer of refractory material, e. g., 35 granular, four inches thick, a clay layer five inches thick beneath the refractory layer, an asbestos layer four inches thick beneath the clay layer, and a concrete foundation twenty-four inches thick, I placed the thermo-couple of the pyrometer at the top of the asbestos layer, nine inches beneath the floor, with the end of the thermo-couple disposed near the center of the oven floor. 40 At this point, the temperature effect on the thermo-couple provided an accurate indication of the 45 temperature conditions within the oven. With the thermo-couple positioned as hereinabove described and coking coal tar pitch of 400° F. melting point, I found that the pulling of the oven, i. e., the quenching of the coke in the oven fol- 50 55

lowed by the removal of the coke, when the pyrometer showed a temperature within the range of from 900° F. to 1100° F., and preferably within the range of from 900° F. to 1000° F., the charge was completely coked and firm, dense coke resulted. Water was introduced into the oven in amount sufficient to quench the coke, e. g., 85 gallons of water per ton of coke produced, and the oven thus cooled to a temperature of 800° F. for the reception of the next charge.

In the drawing—

Fig. 1 is a vertical section through a beehive oven for coking coal tar pitch, equipped with a thermo-couple beneath the floor of the oven, 15 and

Fig. 2 is a plan section of the oven of Fig. 1 taken in a horizontal plane passing through line 2-2 of Fig. 1.

In the drawing, reference numeral 1 indicates a concrete foundation which may be approximately twenty-four inches thick for a beehive oven 2. Disposed on the foundation 1 is a layer, approximately four inches thick, of loose asbestos 3 tamped into place on top of the concrete foundation 1. On top of the asbestos layer 3 is a clay layer 4, approximately five inches thick. The floor proper 5 of the oven 2 is constituted of a refractory layer, e. g., ganister, approximately four inches thick. As customary, the beehive oven 2 is provided with a charging hole 6 which may be closed by means of a suitable closure (not shown), a flue 7 through which products of combustion may escape from the oven, and an opening or port 8 through which air or other oxygen-containing gas may be admitted to support combustion of the volatile matter during the beehive coking of the pitch, and after quenching of the coke in the oven, the coke may be withdrawn. The quenching water may be introduced through charging hole 6.

A thermo-couple well 9 is disposed on top of the asbestos layer 3. This well may be formed by placing a suitable pipe, as shown in Fig. 2, with the end 11 of the pipe disposed near the center of the floor of the oven. A thermo-couple is disposed in the well 9. With the thermo-couple positioned as hereinabove described, an accurate representation of the temperature conditions within the oven, particularly in the floor thereof, is given by the pyrometer with which the thermo-couple communicates.

In coking hydrocarbon material in an oven, as shown in the drawing, the charge is withdrawn from the hot oven when the pyrometer chart, on which the temperatures to which the thermo-couple is subjected are recorded, shows a temperature within the range of from 900 to 1100° F., preferably within the range of from 900 to 1000° F. With 400° F. melting point coal tar pitch and a charge of six tons of pitch in an oven of the type shown on the drawing, the coking time required will be approximately 52 hours. This represents a reduction of the order of 8 hours in coking time as compared with the coking time heretofore customarily employed in coking coal tar pitch of like melting point. Furthermore, an increase in the amount of high quality coke produced results from the practice of my invention and the coke formed is of uni-

formly good quality, the production of spongy, foamy coke being eliminated.

Since certain changes may be made in carrying out the above process without departing from the scope of the invention, it is intended that all matter contained in the above description shall be interpreted as illustrative and not in a limiting sense.

What is claimed is:

1. The process of coking successive charges of pitch in a beehive oven heated to a temperature such that the floor of the oven is at a temperature of from about 600° F. to about 800° F. which comprises introducing a charge of coal tar pitch into said heated oven, introducing a combustion-supporting gas into said oven to burn volatile matter in said coal tar pitch and to heat the latter to form coke, quenching the coke when the floor of said oven reaches a temperature of from about 1500° F. to about 2000° F. thereby resulting in a lowering of the temperature of the oven, removing the coke when the temperature at the floor of the oven reaches a temperature of from about 600° F. to about 800° F. and then introducing the next charge of coal tar pitch into the oven, the introduction of the said charge of coal tar pitch resulting in a further lowering of the temperature at the floor of the oven to a temperature of from about 400° F. to about 600° F.

2. The process of coking successive charges of pitch in a beehive oven heated to a temperature such that the floor of the oven is at a temperature of from about 600° F. to about 800° F. which comprises charging coal tar pitch into said heated oven, admitting air into said oven to burn a portion of said coal tar pitch, until said oven floor reaches a temperature falling within a predetermined range of from about 1500° F. to about 2000° F., and the pitch is coked, quenching the resultant coke until the floor of the oven reaches a predetermined temperature within the range of from about 600° F. to about 800° F., removing the coke from said oven and introducing the next charge of coal tar pitch into said oven.

3. The process of coking coal tar pitch in a beehive oven having a refractory floor approximately four inches thick, a layer of clay approximately five inches thick beneath the floor, a layer of asbestos approximately four inches thick beneath the layer of clay, and a concrete foundation approximately twenty-four inches thick beneath the layer of asbestos, the steps which comprise introducing coal tar pitch into said beehive oven which has been heated by a previous coking operation, the temperature of said oven at the beginning of the introduction of said coal tar pitch indicated on a thermo-couple placed on top of the layer of asbestos and positioned approximately in the center of the floor of the oven being about 800° F., coking the coal tar pitch in the oven by burning a portion thereof by means of air admitted thereto until the said thermo-couple indicates a temperature within the range of from about 900° F. to about 1000° F. and the pitch is coked, immediately thereafter introducing water into the oven in an amount sufficient only to quench the coke and to reduce the temperature indicated on said thermo-couple to about 800° F., and then removing the coke.

DANIEL TOLLIE SMITH. 70